

## UNITED STATES PATENT OFFICE

2,159,124

## ALLOY

Jesse O. Betterton, Metuchen, Albert J. Phillips,  
Plainfield, and Albert A. Smith, Jr., Metuchen,  
N. J., assignors to American Smelting and Re-  
fining Company, New York, N. Y., a corpora-  
tion of New Jersey

No Drawing. Application May 20, 1937,  
Serial No. 143,756

2 Claims. (Cl. 75—167)

This invention relates to lead alloys and pro-  
vides certain alloys of calcium, lead and tin  
which have been found to possess properties  
making them of particular importance in the  
5 manufacture of battery grids and sheathing for  
electrical conductor cables.

The alloys of the invention consist of 0.01%  
to 0.1% calcium, 0.35% to 1.75% tin and the bal-  
10 ance lead, it being understood that the alloys,  
while essentially ternary compositions, may con-  
tain minor impurities within the scope of the in-  
vention as defined in the appended claims.

The alloys may be readily compounded in any  
15 of several manners, one of the simplest being to  
melt the lead in an ordinary cast iron kettle and  
stir in the requisite tin and calcium, the latter  
being added in the form of a calcium-lead alloy.

The advantages accompanying the use of the  
20 alloys of the invention in the manufacture of  
such products as battery grids and cable sheath-  
ing are readily apparent from a consideration of  
the properties of the new alloys.

Thus, the alloys of the invention are eminently  
25 more stable upon remelting than are the calcium-  
lead alloys recently advocated for battery grids  
as a substitute for antimonial grid metal. This is  
well illustrated from the following tabulated re-  
30 sults of drossing tests conducted on several of  
the new alloys by melting 1000 grams of the  
alloy in a special machine equipped with a re-  
volving paddle which swept the surface of the  
molten metal (350° C.—360° C.) at exactly 100  
35 R. P. M. for 30 minutes after which the remain-  
ing metal was skimmed clean, cast and chemi-  
cally analyzed. A typical result from a like test  
on a binary calcium-lead alloy is included for  
the purpose of comparison.

| 40 | Alloy composition before<br>dross test | Alloy composition after<br>dross test | Per cent<br>Ca re-<br>tained |
|----|----------------------------------------|---------------------------------------|------------------------------|
|    | Pb, 0.065% Ca.                         | Pb, 0.010% Ca.                        | 15                           |
|    | Pb, 0.062% Ca, 0.46% Sn.               | Pb, 0.038% Ca, 0.46% Sn.              | 58                           |
|    | Pb, 0.058% Ca, 0.95% Sn.               | Pb, 0.035% Ca, 0.95% Sn.              | 60                           |
| 45 | Pb, 0.037% Ca, 1.20% Sn.               | Pb, 0.029% Ca, 1.14% Sn.              | 78                           |

The ability of the calcium-lead-tin alloys of  
the invention to retain a much larger percentage  
of their calcium upon remelting than is the case  
50 when remelting binary calcium-lead alloys is of  
considerable importance when one considers the  
large amounts of metal that must be remelted  
in many processes as, for example, in manufac-  
turing battery grids where the weight of metal  
55 to be remelted and returned to the process often  
approximates the weight of satisfactory grids  
produced. Hence, it will be appreciated that  
while calcium-lead alloy grids may be considered  
to constitute an improvement over antimonial  
55 grids in that they are said not to accelerate

sulphation or cause self-discharge of the battery,  
the calcium-lead-tin alloys of the invention are  
a decided improvement over the calcium-lead  
5 grids in that they are vastly more stable upon  
remelting and in this respect more closely ap-  
proach antimonial grid metal which may be re-  
peatedly remelted with very little change in  
chemical composition.

In addition to the marked increase in stability  
of the calcium-lead-tin alloys of the invention  
over alloys of calcium-lead, the presence of the  
tin has been found to impart increased tensile  
10 strength. Thus a cast alloy consisting of 0.054%  
calcium, 1% tin and the balance lead exhibited  
a tensile strength of approximately 8000 lbs./sq.  
in. as compared to 5500 lbs./sq. in. for a cast  
alloy consisting of 0.057% calcium and the bal-  
15 ance lead. Apparently, the tin exerts a strength-  
ening effect by stiffening the matrix. On ex-  
truded material, tensile strength values of about  
6500 lbs./sq. in. were obtained for the calcium-  
lead-tin alloy but because of the technique em-  
ployed in the tests this figure should not be con-  
sidered as representing the maximum obtainable.  
Fatigue strength was found to be approximately  
20 1700 lbs./sq. in. for 20 million cycles at 2000  
R. P. M.

It will thus be apparent to those skilled in the  
art that the characteristics of the improved alloys  
fit them for such special uses as cable sheathing  
25 and battery grids. In connection with the latter  
use it may be pointed out that the new alloys  
retain their hardness upon remelting and lend  
themselves to grid manufacture by punching or  
stamping methods which some manufacturers  
30 have long felt to be desirable but to which anti-  
monial lead is not easily adapted by reason of  
the fact that while it can be rolled into sheet  
material, the sheets are softer and less rigid than  
the cast metal and the normally rolled sheet  
35 actually softens with time unless the tendency  
be overcome by heat treatment thereby making  
the process commercially unattractive.

While the beneficial properties which charac-  
terize the improved alloys of the invention are  
exhibited, to a more or less degree, by any com-  
position falling within the limits hereinbefore  
specified (0.01% to 0.1% Ca, 0.35% to 1.75% Sn,  
balance Pb), it has been found that a tin range  
of between 0.5% and 1.25% is preferable for most  
50 uses.

What is claimed is:

1. An alloy consisting of 0.01% to 0.1% cal-  
cium, 0.35% to 1.75% tin, and the balance lead.
2. An alloy consisting of 0.01% to 0.1% cal-  
cium, 0.5% to 1.25% tin, and the balance lead.

JESSE O. BETTERTON.

ALBERT J. PHILLIPS.

ALBERT A. SMITH, JR.